

# UNITED STATES PATENT OFFICE.

JAMES H. SHELDON, OF ZANESVILLE, OHIO.

## WATERPROOFING CLOTH.

SPECIFICATION forming part of Letters Patent No. 337,528, dated March 9, 1886.

Application filed September 15, 1885. Serial No. 177,177 (No specimens.)

*To all whom it may concern:*

Be it known that I, JAMES H. SHELDON, of Zanesville, in the county of Muskingum and State of Ohio, have invented certain new and useful Improvements in Waterproofing Cloth, of which the following is a full, clear, and exact description.

The object of this invention is to provide an improved method of waterproofing cloth made wholly or in part of wool, by the use of which the cloth will be made impervious to water without having its color affected or being injured in any way.

The invention consists in the method of waterproofing cloth hereinafter fully described, and then claimed.

In carrying my invention into practical effect I put a quart of hot soft water in a vessel, then add a half-ounce of gum-arabic and a half-ounce of fine table-salt, (rock-salt is preferred,) and heat the mixture until the gum-arabic is fully dissolved. The solution is then poured into a vessel containing three quarts of hot soft water in which fourteen ounces of the best alum has been dissolved, and the mixture is thoroughly stirred. The cloth to be waterproofed is then immersed in this solution until saturated, is well handled and aired for about twelve or fourteen minutes, and is hung up to drain for twenty-five or thirty minutes. The cloth is then

again immersed in the hot solution for six or eight minutes, and is again hung up for about six or eight minutes. The cloth is then immersed for six or eight minutes in a warm solution of one ounce of Spanish whiting and four ounces of the best prepared chalk dissolved in a gallon of hot soft water. The cloth is then well handled and aired, and hung up to dry, care being taken to hang smooth. The cloth when dry is well brushed with the nap, and is ready for market or use, or, if desired, the cloth can be pressed and finished in the same manner as other cloths.

The invention can be applied to cloth in the web or to cloth made into garments.

Having thus described my invention, I claim as new and desire to secure by Letters Patent

The method of waterproofing cloth here set forth, which consists in saturating the cloth one or more times in a hot solution of gum-arabic, table-salt, and alum dissolved in hot soft water, then handling and airing it, then hanging it up to drain, then saturating the cloth in a warm solution of Spanish whiting and prepared chalk, then handling and airing it, and then hanging it up to dry, all substantially as described.

JAMES H. SHELDON.

Witnesses:

HOWARD ASTON,  
MARGARET SLOAN.